

Feb. 24, 1942.

L. A. BANNON

2,274,031

INSULATED ELECTRICAL CONDUCTOR

Filed Feb. 25, 1938



Fig. 1



Fig. 2

Fig. 3

Lewis A. Bannon Inventor

By P. L. Young Attorney

## UNITED STATES PATENT OFFICE

2,274,031

## INSULATED ELECTRICAL CONDUCTOR

Lewis A. Bannon, Roselle, N. J., assignor to Standard Oil Development Company, a corporation of Delaware

Application February 25, 1938, Serial No. 192,480

5 Claims. (Cl. 174—25)

This invention relates to improved insulated electrical conductors and methods of manufacturing same and more particularly it relates to electrical conductors insulated with synthetic oils derived from lower molecular weight aliphatic hydrocarbons.

In the construction of insulated electrical conductors, it is frequently desirable to use an oil as one of the primary insulating mediums, particularly in the case of cables in which a single or stranded electrical conductor has an outer coating such as a lead sheath, there being an insulating space between the conductor and the sheath; in such a case, this insulating space is generally filled with an oil alone, small solid objects being used as spacers to keep the conductor properly positioned in the center of the surrounding lead sheath, or else the conductor is wrapped with paper and after covering with a lead sheath, the insulating oil is forced in under pressure until it has thoroughly impregnated all the paper wrapping and has filled any interior interstices. The oil to be used for such purposes must meet various requirements as to certain physical properties in addition to having satisfactory resistivity and other electrical properties. For example, when the conductor is first wrapped with paper and then impregnated with the oil, it is essential that the oil have great penetrating power at the temperature being used for the impregnation and yet it is desirable that the oil become extremely viscous or practically solidified at atmospheric (operating) conditions. Under such circumstances it is desirable to use an oil having a very low V. I. (viscosity index). This V. I. is a measure of the viscosity-temperature relationship of an oil; a high V. I. oil shows relatively little change in viscosity for a given change in temperature, but a low V. I. oil shows a relatively great change in viscosity for a given change in temperature. This V. I. test is explained in an article entitled, "Viscosity Variations of Oils with temperature," by Dean and Davis, Chem. & Met., vol. 36, pg. 618-9 (October, 1929).

On the other hand, when it is desired to use as cable insulation an oil which will not change very much in fluidity or viscosity over a fairly wide temperature range, such as the upper and lower limits of atmospheric temperature, it is desirable to use an oil having substantially higher

V. I., such as between the approximate limits of 75 and 120.

According to the present invention, electrical conductors may be insulated with either relatively high V. I. or low V. I. synthetic oils made according to a process which is adaptable to the production of either type of oil, depending upon the intended use. It is preferred to make and use the low V. I. oils, as there has heretofore been a substantial scarcity of materials which are satisfactory for this purpose.

Broadly, the invention comprises treating low molecular weight normally liquid polymers of normally gaseous olefines, particularly iso-olefines, with an acid-reacting halide catalyst of the Friedel-Crafts type, such as aluminum chloride, boron fluoride and the like, at a temperature between the approximate limits of —50° C. and 120° C., preferably between about 0° and 100° C. Suitable polymer raw materials include di-isobutylene, trisobutylene, or other higher polymers. Similar polymers of other iso-olefines, such as 2-methyl butene-1, may be used, and also co-polymers, such as those of iso-olefines combined with normal olefines, e. g., a co-polymer of iso-butylene and normal butylene. When these various polymers are treated alone with a catalyst, the resultant oil has a relatively low V. I., generally below 10, and they may be as low as —200 or lower.

Isobutylene is an unsaturated hydrocarbon of the formula  $C_4H_6$ , having one unsaturated linkage between carbon atoms. Accordingly, iso-butylene dimer produced from two isobutylene molecules has eight carbon atoms; trimer has twelve carbon atoms; tetramer has sixteen carbon atoms; and pentamer has twenty carbon atoms. These may be called the low polymers, and are the preferred raw materials for the present invention.

On the other hand, if these low molecular weight polymer raw materials are treated with a catalyst in the presence of a substantial amount of olefine monomer, preferably an iso-olefine such as iso-butylene, 2-methyl butene-1, etc., at similar temperature, a resultant oil is produced which has a substantially higher V. I. in the range of from 75 up to 140 or more. The yield and the V. I. of the oil will depend greatly on the proportion of monomer and polymer raw material,

as well as upon the temperature and the amount and type of catalyst. Generally the proportion of monomer, such as iso-butylene, should not be more than 3 times the weight of the dimer or other low molecular weight polymer used.

Some general requirements which apply both to the high V. I. oils and the preferred low V. I. oils are that they should have a molecular weight between the approximate limits of 300 or 400 and about 5000 and that their Saybolt viscosity at 100° F. should not greatly exceed about 20,000 seconds and preferably should be not more than 5000. Due to their characteristic method of manufacture of these oils, they all have a relatively low pour point, e. g. between about 0° and -25° F., because they are wax-free and no dewaxing is required, even though they may have the high viscosity mentioned above. They have very high penetration and spreading power.

The preferred type of oil, namely, the low V. I. oils, should generally have a Saybolt viscosity of between the approximate limits of 35 and 200 seconds at 210° F. and should generally have a viscosity of over 100 and preferably over 400 seconds at 100° F.

On the other hand, the high V. I. oils can tolerate a substantially higher viscosity at 210° F., namely, between the approximate limits of 50 and 1000 seconds, while their viscosity at 100° F. will generally not be below 400 and is preferably between about 1000 and 10,000.

As catalyst, it is also possible to use complexes

For the sake of illustration, but without intending to limit the invention thereto, some experimental data are given herebelow.

Table 1 sets forth data on the manufacture of low V. I. oils by polymerization of diisobutylene alone, whereas Table 2 gives data on the treatment of isobutylene with diisobutylene (referred to in the table as dimer) with the resultant formation of oils having a V. I. ranging from about 90 to 140.

TABLE 1  
Low V. I. cable oils

| 15 | Reactant       | Catalyst                                        | Reaction temp. | Oil characteristics |          |       |
|----|----------------|-------------------------------------------------|----------------|---------------------|----------|-------|
|    |                |                                                 |                | Vis./100            | Vis./210 | V. I. |
| 20 | Diisobutylene. | BF <sub>3</sub> -H <sub>2</sub> O               | °C.            | 10                  | 138.9    | 39.7  |
|    | Do             | BF <sub>3</sub> -H <sub>2</sub> SO <sub>4</sub> |                | 0                   | 17,500   | 173.6 |
|    | Do             | AlCl <sub>3</sub>                               | 100 to 110     |                     | 352.7    | 46.5  |
|    | Do             | AlCl <sub>3</sub>                               | 25             |                     | 304.5    | 45.3  |
|    | Do             | BF <sub>3</sub>                                 | -40 to -50     |                     | 444      | 50.6  |

Such low V. I. oils produced by polymerizing diisobutylene under the conditions indicated spread over five times more surface than a mineral oil of the same viscosity at 100° F. placed on a highly polished surface for a given length of time. Therefore, these oils are particularly adapted for penetrating into interstices of a fibrous paper or other wrapping material used in making insulated electrical cables.

TABLE 2  
High V. I. cable oils

| Percent isobutylene | Dimer | Temp.      | Catalyst                          | Oil characteristics |          |       |
|---------------------|-------|------------|-----------------------------------|---------------------|----------|-------|
|                     |       |            |                                   | Vis./100            | Vis./210 | V. I. |
| 50                  | 60    | °C.        |                                   |                     |          |       |
| 66.3                | 22.3  | 0          | BF <sub>3</sub>                   | 4,600               | 403      | 140   |
| 66.3                | 33.3  | 0          | AlCl <sub>3</sub>                 | 11,705              | 385.2    | 94    |
| 66.3                | 33.3  | -15        | AlCl <sub>3</sub>                 | 7,938               | 1,049    | 137   |
| 66.3                | 33.3  | 0          | BF <sub>3</sub> -H <sub>2</sub> O | 410                 | 66       | 125   |
| 50                  | 60    | -40 to +50 | BF <sub>3</sub>                   | 5,551               | 288      | 107   |

of aluminum chloride or boron fluoride or other materials, for instance, a solution of excess boron fluoride in complexes of boron fluoride and water, and boron fluoride and sulfuric acid.

The exact manner of carrying out the polymerization or copolymerization may be varied somewhat. For instance, the catalyst, alone or dispersed in a solvent or diluent, may be added to the polymer or copolymer raw material, such as diisobutylene, alone or in admixture with the mono-isoolefin, such as isobutylene, and/or in the presence of an additional liquid serving as solvent or diluent, such as liquefied propane or butane. When the dimer is to be copolymerized with the monomer, better control of the reaction is obtained by first dissolving or suspending the catalyst, such as boron fluoride or aluminum chloride, in the less reactive of the two raw materials, namely, the diisobutylene, and then feeding the monomer isobutylene into the dispersion of catalyst in the dimer. The reason for this advantage is probably that it permits a quicker absorption of the heat of reaction and prevents the possibility of rapid reaction with the resultant liberation of tremendous quantities of heat and possible explosion. Furthermore, the better control of the reaction has the advantage of producing a product having a narrower molecular weight spread and therefore the product is more uniform.

The high V. I. cable oils produced as indicated in Table 2 have good spreading properties and low pour point and are, therefore, superior to natural paraffinic oil distillates of corresponding viscosity, because the paraffinic oils generally owe their high V. I. to the presence of waxy constituents which tend to give the oil a relatively high pour point and yet if the oil is dewaxed in order to produce a satisfactorily low pour point, the V. I. is correspondingly reduced.

For the sake of illustration, several modifications of insulated electrical conductors are shown in the accompanying drawing.

Fig. 1 shows a longitudinal view of an electrical conductor 1, surrounded by an outer protective layer, such as lead sheath 2, has an intermediate spiral wrapping of paper 3 which has been impregnated with the preferred synthetic oil insulating medium. In practice, either the paper is impregnated with this oil prior to wrapping around the conductor, or, as in the preferred practice, the dry paper is

70 wrapped around the conductor and covered with 75

a lead sheath and then, after evacuating as much as possible of the air, the entire paper wrapping is impregnated by forcing hot oil into one end of the cable until it issues at the other end.

Referring to Figs. 2 and 3, electric conductor 1 is surrounded with an outer protective metal layer, such as lead sheath 2, and by means of any suitable spacing means 4 the conductor is held properly positioned in the center of the lead sheath 2 and then the intervening space between the conductor 1 and sheath 2 is filled with the preferred synthetic oil insulating medium described in the specification.

In the appended claims, when the term "polymer" is used in describing low molecular weight polymers of iso-olefins, it is intended to also include copolymers of iso-olefins with normal olefins.

It is not intended that the invention be limited to any of the specific examples or specific embodiments of the invention which have been given merely for the sake of illustration, nor to any theories given as to the mechanism of the operation of the invention, but only by the appended claims in which it is intended to claim all novelty inherent in the invention as broadly as the prior art permits.

I claim:

1. An insulated electric cable comprising in combination a metallic conductor, a sheath and an insulator member surrounding said conductor within said sheath consisting of a solid insulating member and a submerging insulating oily olefinic polymer produced by polymerization of an isobutylene dimer characterized by fluidity, by a low pour point below about 0° F., by freedom from wax, by a high penetrating and spreading power, by a molecular weight between the limits of approximately 300 and 5,000 and a viscosity index below approximately 0.

2. An insulated electric cable comprising in combination a metallic conductor, a sheath and an insulator member surrounding said conductor within said sheath consisting of a solid insulating member and a submerging insulating oily olefinic polymer produced by polymerization of an isobutylene dimer characterized by fluidity, by a low pour point below about 0° F., by freedom from wax, by a high penetrating and

spreading power, by a molecular weight between the limits of approximately 300 and 5,000, by a viscosity index below approximately 0, by a Saybolt viscosity at 210° F. within the range of approximately 35 to 200 seconds and a Saybolt viscosity at 100° F. above 400 seconds.

3. An insulated electric cable comprising in combination a metallic structure, a sheath and an insulating member surrounding said conductor within said sheath consisting of a fibrous material wrapping around said conductor within said sheath and a submerging body of an insulating oily olefinic polymer produced by polymerization of an isobutylene dimer characterized by fluidity, by a low pour point below about 0° F., by freedom from wax, by a high penetrating and spreading power, by a molecular weight between the limits of approximately 300 and 5,000 and by a viscosity index below approximately 0.

4. An insulated electric cable comprising in combination a metallic structure, a sheath and an insulating member surrounding said conductor within said sheath consisting of a fibrous material wrapping around said conductor within said sheath and a submerging body of insulating oily olefinic polymer produced by polymerization of an isobutylene dimer characterized by fluidity, by a low pour point below about 0° F., by freedom from wax, by a high penetrating and spreading power, by a molecular weight between the limits of approximately 300 and 5,000, by a viscosity index below approximately 0, by a Saybolt viscosity at 210° F. within the range of approximately 35 to 200 seconds and a Saybolt viscosity at 100° F. above 400 seconds.

5. An insulated electric cable comprising in combination a metallic structure, a sheath and an insulating member surrounding said conductor within said sheath consisting of a solid insulating spacer means around said conductor within said sheath and a submerging body of insulating oily olefinic polymer produced by polymerization of an isobutylene dimer characterized by fluidity, by a low pour point below about 0° F., by freedom from wax, by a high penetrating and spreading power, by a molecular weight between the limits of approximately 300 and 5,000 and by a viscosity index below approximately 0.

LEWIS A. BANNON.